

## UNITED STATES PATENT OFFICE.

CARL J. ZAISER, OF MILWAUKEE, WISCONSIN, ASSIGNOR TO AMERICAN METAL PRODUCTS COMPANY, OF MILWAUKEE, WISCONSIN, A CORPORATION OF WISCONSIN.

## ALLOY.

No Drawing.

Application filed May 23, 1921. Serial No. 471,914.

*To all whom it may concern:*

Be it known that I, CARL J. ZAISER, a citizen of the United States, and resident of Milwaukee, in the county of Milwaukee and State of Wisconsin, have invented new and useful Improvements in Alloys, of which the following is a description, reference being had to the accompanying drawings, which are a part of this specification.

10 The object of the invention is to produce a new and improved alloy, superior to existing alloys known as bronzes, by reason of its lightness, cheapness and greater tensile strength, the alloy having a tensile strength

15 equal to that of mild steel and, unlike other bronzes, capable of being forged, rolled, welded, soldered, drawn or otherwise worked in a manner similar to iron or steel. This alloy may be produced in different forms,

20 such as ingots, pigs, billets, bars, etc., for producing sand castings, die castings, rolled material, drawn material, stampings, forgings, drop forgings, and is especially de-

signed for the manufacture of bearings, valves and shafting.

25 The alloy contains the following metals in substantially the following proportions, namely:

|               | Per cent. |
|---------------|-----------|
| Iron-----     | 13 to 60  |
| Copper-----   | 82 to 30  |
| Aluminum----- | 5 to 10   |

30 These metals are melted together and the resultant alloy is one having desirable characteristics of both mild steel and bronzes, as 35 previously pointed out.

I claim:

An alloy consisting of the following ingredients in substantially the following proportions, namely:

|               | Per cent. |
|---------------|-----------|
| Iron-----     | 13 to 60  |
| Copper-----   | 82 to 30  |
| Aluminum----- | 5 to 10   |

40 In testimony whereof I affix my signature. 45  
CARL J. ZAISER.